

Patented Feb. 23, 1926.

1,573,814

## UNITED STATES PATENT OFFICE.

JUDSON A. DE CEW, OF MOUNT VERNON, NEW YORK, ASSIGNOR TO PROCESS ENGINEERS, INC., OF NEW YORK, N. Y., A CORPORATION OF NEW YORK.

### METHOD OF PREVENTING FROTH ON PAPER MACHINES.

No Drawing.

Application filed December 14, 1921. Serial No. 522,841.

To all whom it may concern:

Be it known that I, JUDSON A. DE CEW, a citizen of the Dominion of Canada, residing at Mount Vernon, New York, have invented certain new and useful Improvements in Methods of Preventing Froth on Paper Machines, of which the following is a specification.

I have discovered that the formation of injurious froth on the screens of paper machines is due to two causes, namely, agitation of the stock in the presence of air, and the capacity of the stock to form froth due to the presence in the stock of certain frothing agents.

Both conditions are necessary to the formation of excessive froth. When such froth is formed it is found to contain a lot of pulp fibres, which have been carried in the films of the froth bubbles. These fibres are held in the froth by certain oils which may be found in small quantities either in sulphate or sulphite pulp, or in mill waters containing the waste liquors from the manufacture of these pulps, or the rosin used in making the size may contain a trace of these flotation oils.

These oils cause the fibres to float up into the froth and this does the damage on the paper machine.

I have also discovered means for preventing the formation of this injurious froth.

One means is to add to the paper stock, certain agents which either alter the surface tension conditions or cause some other effect which destroys the flotation properties of the oily impurities.

These means are that class of chemical products which will destroy the flotation properties in the fibres, and is represented by ferrous sulphate ( $FeSO_4$ ). This material is known to the trade as copperas or green crystals, and has been used in paper-making as a substitute for alum in sizing the paper, but with poor success because iron resinate have very little sizing value. My method of using it however, is to first

precipitate the size with aluminum sulphate (alum), forming aluminum resinate, and then add the ferrous sulphate to the stock to destroy the tendency of the pulp to adhere to the froth. The amount used will vary with the amount of froth but as general practice, from two to ten pounds per beater will be sufficient. More might be used if required without injury to the stock but it is not desirable to use an excess, especially in lighter colored papers.

When treated in this manner, no iron resinate are formed, the sizing is not injured and the dangerous froth is not formed. This treatment is especially adaptable to kraft paper and other unbleached paper products.

There are other chemical agents that have a destructive action on the flotation property so while ferrous sulphate is my preferred one, I consider my invention broad enough to cover others.

While I have herein referred to the prevention of injurious froth I do not mean to say that absolutely no froth will be formed but that what froth may be formed will be of such a nature that the fibres will not adhere thereto and therefore will not be floated thereby. Accordingly, my invention consists essentially in the prevention of the formation of injurious froth but is broad enough to cover the conversion of injurious froth into a non-injurious kind by eliminating in the previously described manner the affinity of the froth for the fibres.

What I claim is:

1. A method of decreasing the frothing properties of a paper pulp which has been treated with rosin size and alum, which consists in precipitating soluble frothing ingredients by means of a treatment with a soluble iron salt.

2. The method of claim 1, using ferrous sulphate.

In testimony whereof I have affixed my signature to this specification.

JUDSON A. DE CEW.